

## UNITED STATES PATENT OFFICE.

WILLIAM B. GERO, OF EAST ORANGE, NEW JERSEY, ASSIGNOR, BY MESNE ASSIGNMENTS, TO WESTINGHOUSE LAMP COMPANY, A CORPORATION OF PENNSYLVANIA.

## METHOD OF MANUFACTURING METALLIC FILAMENTARY MATERIAL.

No Drawing.

Application filed January 13, 1921. Serial No. 437,035.

My invention relates to the manufacture of metallic materials adapted to be subjected to high temperatures and it has special reference to a process intended to control the formation of the crystalline structure of a body made from such materials.

In the present state of the incandescent lamp art, it is well known that a metallic material, such as tungsten and similar highly refractory metals, unless specially treated will tend to alter internally when raised to a point of incandescence in a lamp, and that the degree of alteration will depend upon such factors as the size of filament, efficiency at which it is operated, length of service, etc. One such form of alteration is manifested in what is commonly known as "sagging", which is particularly noticeable in filaments of the coiled type or in lamps which are designed to be burned horizontally. The effect of sagging in a coiled filament results in adjacent turns of the wire comprising the helix either being separated or short circuited, and, in the case of a lamp having an uncoiled filament, such as those used for sign-lighting purposes, the sagging of the filament permits it to incline to the vertical instead of projecting horizontally. Such alterations impair the lamp's efficiency, with the consequent early failure of the same.

One of the causes for the sagging of the tungsten coils, when hot, is known to be certain conditions of their crystalline structure. A sag wire is characterized by small crystals or grains. The principal characteristic of non-sag wire is its large-grain structure. The grains should be large as to length and cross section. It is also desirable that the crystals have irregular surfaces so that they may interlock and thus form a more stable structure.

Another form of internal alteration common to metallic filaments is known as offsetting, which consists of a lateral shifting or displacement of one portion of filament with respect to an adjacent portion. It has been proposed to control this structural change by the addition of auxiliary substances which resist off-setting through retardation of grain growth. For this purpose thorium oxide is generally used. For a further explanation of this phenomenon reference may be had to United States Pat-

ent No. 1,180,264, issued to Anton Lederer, April 18, 1916.

I have discovered that some oxides, particularly the alkali oxides and the alkali earths, such as lithium oxide, sodium oxide, calcium oxide, etc., when mixed with a compound of tungsten promote grain growth during the process of manufacturing drawn tungsten, that is, cause the grains or crystals to grow in size rather than retard their growth, as is the case in the particular materials heretofore employed to prevent offsetting. I have also discovered that some of these, such as lithium oxide and sodium oxide, not only cause the crystals to grow in all directions but direct the growth along the axis of the wire so that the crystals are of greater length than width when the filamentary material contains one or more of these oxides. This crystalline structure is valuable because it results in a non-sag wire. Furthermore, I have discovered that other oxides, such as potassium oxide, in addition to causing the crystals to grow in size and directing their growth along the axis of the wire, cause the crystals to take on irregular surfaces and thus interlock, the value of which has been stated above.

It is, therefore, an object of my invention to provide a controllable and simplified process for the production of a non-sag structure in highly-refractory filamentary materials by the addition of suitable metallic oxides, followed by mechanical working.

A special object of the invention is the provision of a process especially applicable to the treatment of tungsten for producing a non-sag structure when the tungsten is drawn into filamentary form.

Although my invention is applicable to producing bodies from refractory metals generally, for the purpose of illustration, I will describe how it may be practiced in producing a tungsten wire possessing non-sag properties developed by the process contemplated by me.

A solution of any soluble salt of the alkali or alkali-earth metals, such as the nitrates, chlorides, silicates, carbonates, etc., is mixed, in certain proportions, with purified and precipitated tungsten trioxide ( $WO_3$ ). If the additive substance be potassium nitrate, 200 cc. of an aqueous solu-

tion containing .8 of a gram of potassium oxide ( $K_2O$ ) is added to a kilogram of tungsten trioxide. This mixture, when dried at  $300^\circ C.$  to  $700^\circ C.$ , contains .08% 5 potassium oxide. It is then subjected to a double-reduction process which consists in reducing the oxide of tungsten by hydrogen at as low a temperature as possible, mixing the reduced material with an equal 10 weight of tungsten trioxide and reducing this mixture by passing it through a furnace having a hydrogen atmosphere at a temperature of about  $600^\circ C.$  to  $800^\circ C.$ . The resultant powder is compressed to form 15 billets or slugs about 16 inches long and  $\frac{1}{4}''$  square. Electric current of about 1600 amperes is passed through this slug to effect a sintering action; at the same time, most of the potassium nitrate is volatilized 20 as potassium oxide and thus removed from the tungsten slug. The slug is then swaged and drawn into wire according to any approved process for producing drawn tungsten wire.

25 From the foregoing it is to be appreciated that the additive substance which is incorporated into the base material may vary, and that the quantity necessary to produce the desired result may likewise vary. I 30 have found that, in certain sizes of filaments, lithium oxide is to be preferred over other compounds of the alkali or alkaline earth metals, and that, for other sizes of filament, potassium oxide appears to be the 35 most satisfactory. For example, in a tungsten wire of 25 mil diameter, such as is used in an incandescent lamp employed as a light source for projection work, lithium oxide promotes a crystalline structure which is 40 found to be very non-sag as compared to an untreated or undoped filament of the same diameter. On the other hand, potassium oxide has been found to give the best results when used in filaments of 10 mil or 45 less in diameter. However, I consider it possible for a single substance to be effective in aiding coarse crystallization in all sizes of wire, providing a suitable process is employed for incorporating the additional 50 substance into the filamentary material. It appears to be largely a matter of rendering patent certain characteristics which are delayed or not present in the various stages of the drawing of the tungsten or filamentary material into sizes of wire suitable for 55 all types of lamps.

It will, therefore, be seen that my invention resides not so much in the quantity or method of adding a given substance 60 capable of exercising control over crystal growth as it is in appreciating that the presence of such a substance exerts such a control which may be utilized in obtaining a beneficial result largely desirable in certain forms of incandescent lamps.

What is claimed is:

1. The method of preparing tungsten powder from which filamentary material may be produced having a definite predetermined grain or crystal structure, which 70 renders the filament resistant to substantial sagging and offsetting when burned at high temperatures which comprises mixing with a tungsten oxide free from compounds deleteriously affecting grain growth, a predetermined quantity of at least one salt of a particular alkali or alkaline earth metal capable of promoting a definite grain or crystal structure in the filament when annealed or burned, and reducing by hydro- 80 gen.

2. The method of preparing tungsten powder from which filamentary material may be produced having an interlocking grain or crystal structure, which comprises mix- 85 ing with a tungsten oxide free from compounds deleteriously affecting grain growth, a predetermined quantity of at least one salt of a particular alkali or alkaline earth metal capable of promoting said grain or crystal 90 structure in the filament when annealed or burned, and reducing by hydrogen.

3. The method of preparing tungsten filaments having a definite predetermined grain or crystal structure therein when burned or 95 annealed which renders the filament resistant to sagging and offsetting, which comprises mixing with tungsten oxide free from compounds deleteriously affecting grain growth, a predetermined quantity of at least one salt of a particular alkali or alkaline earth metal capable of promoting a definite grain or crystal structure in the filament 100 when burned or annealed, reducing by means of hydrogen to obtain a mixture of 105 metallic tungsten and a compound of the alkali metal employed, pressing the powder to form, sintering and mechanically working 110 to filament size.

4. The method of preparing tungsten filaments having an interlocking grain or crystal structure therein when burned or annealed, which comprises mixing with tungsten oxide free from compounds deleteriously affecting grain growth, a predetermined 115 quantity of at least one salt of a particular alkali or alkaline earth metal capable of promoting said grain or crystal structure in the filament when burned or annealed, reducing by means of hydrogen to obtain a 120 mixture of metallic tungsten and a compound of the alkali metal employed, pressing the powder to form, sintering and mechanically working to filament size.

5. The method of preparing tungsten powder from which filaments may be produced having grains or crystals of greater length than width and which have irregular 125 surfaces interlocking with adjacent crystals, which comprises mixing with tungsten oxide 130

free from deleterious compounds affecting grain growth, a predetermined quantity of a compound containing potassium or the like, which is capable of promoting said crystal formation, and reducing by hydrogen.

6. The method of preparing tungsten filaments having grains or crystals of greater length than width and having irregular surfaces interlocking with adjacent crystals, said structure being developed after burning or annealing, which comprises mixing with tungsten oxide free from deleterious compounds affecting grain or crystal growth, a predetermined quantity of a compound containing potassium or the like, capable of promoting said crystal formation, reducing by hydrogen, pressing the powder to form, sintering and mechanically working to filament size.

7. A tungsten base material from which wire may be produced having a definite predetermined crystal or grain formation and which renders the wire resistant to sagging and offsetting, which comprises tungsten powder free from compounds inhibiting the formation of a definite crystal structure and containing a predetermined quantity of a compound containing at least one salt of a particular alkali or alkaline earth metal capable of promoting a definite crystal structure when the powder is fabricated into wire and burned or annealed.

8. A tungsten base material from which wire may be produced having an interlocking crystal or grain formation, which com-

prises tungsten powder free from compounds inhibiting the formation of a definite crystal structure and containing a predetermined quantity of a compound containing at least one salt of a particular alkali or alkaline earth metal capable of promoting said crystal structure when the powder is fabricated into wire and burned or annealed.

9. A tungsten base material from which wire may be produced having grains or crystals of greater length than width and with interlocking contacting surfaces which renders the wire resistant to sagging and offsetting, which comprises tungsten metal free from compounds inhibiting the formation of a definite crystal development but containing a predetermined quantity of a compound of potassium and the like, capable of promoting said crystal formation when the powder is fabricated into wire and burned or annealed.

10. A substantially pure tungsten filament having a definite predetermined grain or crystal formation, said formation having been produced by the addition to tungsten oxide free from compounds inhibiting the formation of a definite grain or crystal structure, of a predetermined quantity of a compound or compounds containing particular alkali or alkaline earth metals selected in accordance with the definite crystal or grain structure desired.

In testimony whereof, I have hereunto subscribed my name this twelfth day of January, 1921.

WILLIAM B. GERO.